

## 1

2,834,724

**METHOD OF ELECTROPLATING PLASTIC ARTICLES**

Abraham Piza Mendes, New York, N. Y.

No Drawing. Application April 26, 1956  
Serial No. 530,964

6 Claims. (Cl. 204—20)

My invention relates to the metal plating of non-metallic substances and has particular relation to the plating of plastic objects with gold or other precious metal utilizing a vapor-vacuum plating procedure as an intermediate step.

The use of a vapor vacuum chamber for the coating of molded plastic articles with such metals as aluminum or the like is well known and commonly employed in the manufacture of inexpensive novelties, etc. Such process deposits a very fine film of metal on the molded plastic, giving the coated article the appearance of being made of solid metal. With conventional methods of plastic molding it is possible to incorporate fine and ornate detail of surface configuration in the molded plastic article, and the thin film of metal deposited by the vapor-vacuum method of plating, retains this fine detail.

It is also well-known to apply gold plating to metals by the conventional electrolytic or gold salts dip methods. Such plating is widely used in the manufacture of costume jewelry, for example, to coat a cast base of copper or bronze with gold. It has been found that fine and ornate surface details cannot be achieved in the case of the metal base, and what detail there may be is appreciably lost when the gold plating is applied.

Because of the ability of plastics such as polystyrene to retain fine surface detail in molding, it would be extremely desirable to plate molded plastic articles with precious metals such as gold for the manufacture of costume jewelry or the like. Up to the present time, there has been no method found, to my knowledge, of plating molded plastic articles directly with gold, because gold will not adhere to plastics nor form thereon by conventional gold-plating methods. The deposition of gold or other precious metals by the vapor-vacuum or sputtering methods is of course impractical commercially because of the tremendous waste of precious materials by this method.

I have found that gold can be deposited on an article of plastic or other non-conductor of electricity, by first coating the article, as by the vapor-vacuum process, with a metal close to gold in the electromotive series. Gold is placed below hydrogen in the electromotive series and has a positive potential in normal metal ion solution; the metal to be applied by the vapor vacuum process must, have a positive potential and it must also be capable of adhering to the surface of the plastic during the deposition of gold.

It is well known that in gold plating, copper affords an excellent plating surface because of its ability to release metallic gold from the plating solution and to provide a surface to which the gold will adhere. Copper is therefore widely used both in electroplating and in gold solution dipping without electricity. It was found, however, that when a molded, plastic article was coated with a thin film of copper by the vapor-vacuum method, and then dipped in the gold solution, the copper peeled off without being replaced by gold. This was the result,

## 2

whether or not current was applied. When current was applied, wide variations in voltage made little difference. The tendency of metallic copper to go into solution, replacing gold ions in that solution, is greater than the adhesion of the metallic copper to the surface with which it is in contact, even when the tendency to go into solution is opposed by an electric current of such direction that it moves metallic (positive) ions to that surface. Furthermore, it was apparent that the copper film was so thin that, having partially replaced the gold ions, there was not sufficient metallic copper remaining to enable the gold ions to lose their charges and become a molecular plating. The gold ions will not lose their charges in contact with the plastic.

15 Antimony and bismuth which have positive electric potentials on the electromotive table, were tried as base coats upon which to plate gold and have proved satisfactory. These metals were applied to the surface of a polystyrene article by the vapor-vacuum method, and a coating of gold was then applied thereupon by electroplating. The antimony and bismuth films adhered to the surface of the plastic article throughout the electroplating process and also adhered well to the plated gold coating. Gold can be deposited on these metals, however, only by electroplating. Since arsenic is grouped with antimony and bismuth in the electromotive series and has similar physical properties, it also could presumably be used, if adequate precautions be taken to prevent the formation of compounds deleterious to health.

30 I have found that the deposition of gold is more rapid, and a coating of better appearance is produced if by the same vapor-vacuum procedure, a coating of copper is applied over the above-stated materials. Conventional electrolytic methods may then be used for the deposition of gold thereon, but the voltage used is preferably lower than that conventionally employed, since high voltages tend to tear or otherwise damage the thin metal films deposited by the vapor-vacuum process.

40 A film of copper deposited by vapor vacuum over a thin film of metal close to gold in the electromotive series may be used to obtain a coating of gold thereon by any of the conventional methods such as "dip," "salt bath," "tumbling," etc. In these methods, the gold ions in solution partially replace the copper film, since no electric current is applied.

45 By this procedure, the base coating of metal acts as a bond between the coating of copper and the surface of the plastic article, preventing the copper film from peeling off in the gold solution. At the same time, the base coating acts as a metal surface to enable the gold ions to lose their charges. The gold ions will not lose their charges in contact with the plastic surface.

50 Other metals were used experimentally for the base coating, but proved unsatisfactory. Lead was used, for example, producing good films on the molded plastic articles. Copper was then deposited on the lead base coating by the same vacuum procedure, forming a fine film coating which retained the surface configuration of the molded plastic. When the coated plastic articles were then placed in a gold plating bath, however, the results were unsatisfactory. Adhesion of the lead to the plastic was insufficient, and copper was removed into the gold solution without being replaced by gold. In the conventional electroplating method, the copper film began to show plated gold at 1½ volts, but loosened and began to peel from the plastic within ten to fifteen seconds.

55 Similar unsatisfactory results were achieved using tin and aluminum in place of lead.

60 Thus the only metals which appear to serve adequately as a base coating beneath the copper coating are those metals which are close to copper in the electromotive

series, namely antimony, bismuth, and arsenic. These metals, in common with copper and the noble metals (gold, silver and platinum) all have positive potentials in contact with solutions in which the metal ion is normal. The metals, antimony, bismuth and arsenic are directly above copper in the electromotive series, and are relatively close to gold. These metals, therefore, will not react with the copper film when dipped in the gold solution, so that adhesion to both plastic and copper is maintained, and the coatings do not peel or loosen. In addition, arsenic, antimony and bismuth have low melting points, so that they may be readily vaporized in the vacuum chamber, and in addition are commercially available and inexpensive.

When arsenic, antimony, or bismuth is used to provide the base coating on the plastic by the vapor vacuum method, it forms a fine adherent film on the surface of the plastic. Copper is then plated over the base coat by the vapor-vacuum method, forming a film which bonds strongly to the base coat and completely covers the base coating. Since copper is used as the intermediate coat, a final gold plating may then be applied either by the conventional dip method or by conventional electroplating methods. In the dip method, the gold ions replace the outer surface of the copper film and then plate the remainder of the copper film before the latter has gone completely into solution. The metal of the base coat adheres to the remainder of the copper film and prevents it from loosening or peeling.

In "Principles of Electroplating and Electroforming" by Blum and Hogaboam, published in 1924, the electromotive series is set forth at page 344. In this series the approximate single potentials of metals toward solutions with normal metal ion concentration, and with a standard based on the normal hydrogen electrode as zero, are listed. The potential of antimony is given as 0.19 volt, arsenic as 0.32 volt, bismuth as 0.33 volt, and copper as 0.34 volt. The metals suitable for use as a base coat on the plastic article thus have positive potentials, but less than 0.34 volt, the potential of copper. From the potentials given, it would be apparent that bismuth would yield better plating results than antimony, and tests have shown this to be true, although satisfactory results were achieved with both bismuth and antimony.

The following is an example of a specific plating procedure in which optimum results were achieved:

The plastic form was made of polystyrene and was first cleaned using a commercial plastic cleaner. The surface of the plastic was then covered with a lacquer compounded to be compatible therewith. Such a lacquer is presently commercially available for vacuum coating with aluminum, and provides better adhesion to the plastic as well as sealing in vapor producing agents such as residual plasticizer.

The metal for producing the base coat was then applied to the plastic. For this purpose, the plastic article was placed in a vacuum chamber, and pure bismuth contained in a molybdenum crucible was also placed in the chamber. The crucible was heated to a dull red by the passage of an electric current therethrough. As the bismuth vaporized, a good film was formed on the plastic article, under a vacuum of approximately one-half micron.

A coating of copper was then formed over the bismuth film by the same vacuum chamber procedure just described, except that the vacuum employed to volatilize the copper was approximately  $\frac{1}{10}$  micron, and the molybdenum crucible was heated to white heat.

The coated article was then placed in a commercial electrolyte solution of gold salts, and a voltage of 1.5 to 2.0 volts applied to the electrodes. A plating of gold adhered to the copper film with the bismuth film as a base. The gold plate was sufficiently adherent to withstand polishing with silver polish.

A plastic article with a base coat of bismuth and a second coat of copper (applied by the vapor vacuum method) was also plated with gold by the conventional salt water process. The article was placed in a porous cup containing a solution of gold salts. The porous cup was placed in a larger vessel containing a solution of sodium chloride and a strip of zinc was suspended in the sodium chloride solution. Gold is then deposited on the article which becomes the cathode of a cell of which the anode was the zinc strip.

While the invention has been described heretofore in terms of achieving a gold plating, it applies equally to a plating of any noble metal, namely silver, platinum or gold. In addition to polystyrene, articles made of other rigid plastics, such as acrylic resins, may be plated by the methods described herein.

What is claimed is:

1. A method of coating a plastic article with a noble metal, which comprises the steps of forming on said plastic article in a vapor vacuum chamber a thin film base of a metal selected from the group consisting of antimony, bismuth and arsenic, and then coating said article with the noble metal by electrodeposition.

2. A method according to claim 1 in which said noble metal is gold.

3. A method of coating a non-porous plastic article with an outer plating of a noble metal, which comprises the steps of vapor depositing on said plastic article a thin film base coating of metal selected from a group consisting of arsenic, antimony and bismuth, then vapor depositing over said base coating an adhering thin film coating of copper, and finally plating the copper coating with a coating of noble metal by electrodeposition.

4. A method according to claim 3 in which the noble metal is gold.

5. A method of coating a molded non-porous plastic article with an outer ornamental plating of a noble metal, which comprises the steps of forming on said plastic article in a vapor-vacuum chamber a thin film base coating of bismuth then forming over said base coating in a vapor-vacuum chamber an adhering thin film coating of copper, and finally plating the copper coating with a coating of gold by electrodeposition, the gold plating adhering to the copper coating.

6. A method of plating a molded plastic article having ornate surface configurations with an adhering outer ornamental coating of a noble metal sufficiently fine to retain the details of said surface configuration, said method comprising the steps of coating said plastic article by evaporation with a fine base coating of a metal selected from the group consisting of arsenic, antimony, and bismuth, then applying by evaporation an adhering intermediate conductive coating over the base coating, the intermediate coating comprising a thin film of copper, and finally providing the plastic article with a thin outer adhering coating of the noble metal by electrodeposition of the noble metal on the intermediate coating.

References Cited in the file of this patent

UNITED STATES PATENTS

|           |                 |                |
|-----------|-----------------|----------------|
| 887,482   | Lammers et al.  | May 12, 1908   |
| 1,548,432 | Belous          | Aug. 4, 1925   |
| 2,133,995 | Lukens          | Oct. 25, 1938  |
| 2,333,534 | Lang            | Nov. 2, 1943   |
| 2,383,311 | Hein            | Aug. 21, 1945  |
| 2,423,476 | Billings et al. | July 8, 1947   |
| 2,439,983 | Morgan et al.   | Apr. 20, 1948  |
| 2,482,054 | Colbert et al.  | Sept. 13, 1949 |
| 2,501,737 | Porter          | Mar. 28, 1950  |
| 2,680,699 | Rubin           | June 8, 1954   |
| 2,702,259 | Sommer          | Feb. 15, 1955  |